

July 1, 1941.

R. C. BOUR

2,247,347

BRIGHT COPYING HECTOGRAPH BLANKET

Filed Feb. 19, 1940

*Fig. 1.*



*Fig. 2.*



Inventor:  
By Robert C. Bour,  
Zalel Carlson, Fitzbaugh & Wells  
Attorneys

## UNITED STATES PATENT OFFICE

2,247,347

## BRIGHT COPYING HECTOGRAPH BLANKET

Robert C. Bour, Chicago, Ill., assignor to Ditto, Incorporated, Chicago, Ill., a corporation of West Virginia

Application February 19, 1940, Serial No. 319,698

5 Claims. (Cl. 41—31.6)

The invention relates to bright copying hectograph blankets.

An object of the invention is to provide hectograph pads of increased toughness, higher copying strength and freedom from sweating.

According to the application of William Hoskins, Jr., entitled Means for and method of duplicating, filed December 20, 1939, Serial No. 310,108, the copy strength of hectograph blankets can be increased considerably by incorporating in the hectograph composition an oil such as a mineral oil or a glyceride of a fatty acid which is not soluble in the constituents of the hectograph mass. However, hectograph masses of this type have been known to sweat very considerably. While this sweating does not render these hectograph blankets valueless, it is a feature which desirably should be eliminated.

A primary object of the invention is, therefore, to provide an improved hectograph blanket over the hectograph blankets described in the Hoskins application Serial Number 310,108.

I have discovered that if an ester of a dihydric alcohol such as glycol oleate, glycol stearate, and di-ethylene glycol laurate, is incorporated in the hectograph mass in quantities from about 2 to 15%, an appreciable increase in copy strength is achieved without objectionable sweating.

Other objects and advantages of the invention will become apparent as the following detailed description progresses, reference being had to the accompanying drawing wherein

Fig. 1 is a sectional elevation of a hectograph pad constituting a preferred embodiment of this invention; and

Fig. 2 is a sectional elevation of a modified hectograph pad.

In Fig. 1 of the drawing, the reference character 1 designates a copy mass comprising a gelatinous composition having dispersed therein droplets or particles of an ester of a dihydric alcohol. The copy mass is secured to a backing 3 of paper, cloth or other suitable material, by means of a bonding layer 2 which may be any of the usual bonding compositions such as linseed oil, fish oil or the like, which are commonly used in the hectograph art to obtain increased adhesion of a copy mass to a backing.

The bonding layer is not essential and may be eliminated, however, with less satisfactory results. This modification is shown in Fig. 2, wherein the reference numeral 1 represents the copy mass containing the ester secured directly to the backing 2.

The copy mass embodied in the present inven-

tion comprises a gelling agent such as glue or gelatin, a water soluble softener such as glycerine, invert sugar, sodium lactate, preferably a hardener such as chrome alum or other protein precipitant, water, and an ester of a dihydric alcohol intimately admixed with the other ingredients as droplets or particles of microscopic or colloidal size.

To illustrate the invention, the following formulas of suitable hectograph compositions are given:

|  | 15                         | Parts by weight |     |     |     |     |     |
|--|----------------------------|-----------------|-----|-----|-----|-----|-----|
|  |                            | I               | II  | III | IV  | V   | VI  |
|  | Gelatin                    | 30              | 30  | 30  | 30  | 30  | 30  |
|  | Water                      | 45              | 45  | 45  | 45  | 45  | 45  |
|  | Glycerin                   | 370             | 375 | 440 | 375 | 440 | 375 |
|  | Invert sugar               | 65              | 65  | —   | 65  | —   | 65  |
|  | Sodium lactate             | 30              | —   | —   | —   | —   | —   |
|  | Sodium citrate             | —               | 10  | —   | —   | —   | —   |
|  | Glycol stearate            | —               | —   | —   | —   | 5   | —   |
|  | Glycol oleate              | 10              | 10  | 15  | —   | 5   | —   |
|  | Di-ethylene glycol laurate | —               | —   | —   | —   | —   | 5   |
|  | Glycol oleate              | —               | —   | —   | —   | —   | —   |
|  | Chrome alum                | .02             | .02 | .02 | —   | —   | —   |

The ingredients are mixed together and heated in a water bath with vigorous agitation so that the glycol ester is emulsified or so finely dispersed in the composition that it will not settle out when standing. The dispersion so formed is coated on the backing and allowed to gel, forming the hectograph blanket. The glycol ester is present in the gelled hectograph mass as the discontinuous phase of a colloid system. This system is sometimes called an oil in water type emulsion or oil in water type dispersion, depending upon whether the glycol ester is a liquid or a solid.

Copies are prepared from the hectograph pad of the invention in the usual manner. A design 40 is formed on a copy paper by writing or typing with an ink made of water or alcohol soluble dyes. The design is then contacted with the gelatinous copy surface of the pad, whereupon the dye is largely transferred to the composition giving the design in mirror reverse. Copies are then made by contacting sheets of paper with the design on the hectograph copy mass. It will be found that a large number of copies of high color intensity can be obtained.

50 While it is not desired to be limited to any theory regarding the mechanism of the action giving the high color intensity, it is believed that the dyes deposited on the composition in the process of duplicating will be loosely bound by powers of surface activity in the interphase between the

dispersed water insoluble particles and the continuous phase of the hydrophilic composition. Therefore, the dye will be retained on or near the surface of the composition, thus being more readily available for copying purposes than would otherwise be the case.

While I have shown and described certain embodiments of my invention, it is to be understood that it is capable of many modifications. Substitution of equivalent materials and changes in the proportions may be made without departing from the spirit and scope of the invention as described in the appended claims, in which it is my intention to claim all novelty inherent in my invention as broadly as possible, in view of the prior art.

I claim:

1. A hectograph blanket comprising a copy mass of a hydrophilic gel containing a water insoluble ester of a dihydric alcohol.
2. A hectograph blanket comprising a backing

having thereon a copy mass of a hydrophilic gel containing a water insoluble ester of a dihydric alcohol dispersed in the copy mass in the form of minute particles.

5. 3. A hectograph blanket comprising a backing having thereon a copy mass of a hydrophilic gel containing glycol oleate dispersed in the copy mass in the form of particles of at least microscopic size.

10 4. A hectograph blanket comprising a backing having thereon a copy mass of a hydrophilic gel containing glycol stearate dispersed in the copy mass in the form of particles of at least microscopic size.

15 5. A hectograph blanket comprising a backing having thereon a copy mass of a hydrophilic gel containing diethylene glycol laurate dispersed in the copy mass in the form of particles of at least microscopic size.

20 ROBERT C. BOUR.